

June 21, 1955

L. A. ROE

2,711,248

CONCENTRATION OF IRON ORES

Filed June 1, 1951

2 Sheets-Sheet 1



Inventor

LAWRENCE A. ROE

By

J. R. Harris

Attorney

June 21, 1955

L. A. ROE

2,711,248

CONCENTRATION OF IRON ORES

Filed June 1, 1951

2 Sheets-Sheet 2

Fig. 2.



Inventor

LAWRENCE A. ROE

By

S. R. Harris

Attorney

# United States Patent Office

2,711,248

Patented June 21, 1955

1

2,711,248

## CONCENTRATION OF IRON ORES

Lawrence A. Roe, Negaunee, Mich., assignor to Jones & Laughlin Steel Corporation, Pittsburgh, Pa., a corporation of Pennsylvania

Application June 1, 1951, Serial No. 229,345

6 Claims. (Cl. 209—39)

This invention relates to a process for concentrating magnetic iron ores and is more particularly concerned with the concentration of low grade magnetic iron ores.

The low grade iron ores to which this invention is primarily directed are siliceous magnetites in which the predominantly silica gangue is intimately associated with the magnetite particles. Such ores may contain iron in amounts from 26% up to perhaps 36% and silica in amounts ranging up to 43% or 44%. The iron is predominantly in the form of magnetite, the proportion of this form reaching 88% or 89%; the balance is principally hematite. Such ore may be concentrated to some degree by conventional wet or dry magnetic processes. However, it is quite generally impracticable and in many cases impossible by conventional processes to recover an economic proportion of the iron and reduce the silica content of the concentrate to a tolerable figure. The difficulty appears to lie in the intimate association of silica particles with magnetite particles. Magnetic separation or concentration processes require that the ore be first ground to a particle size small enough to disengage or unlock the particles of silica from those of magnetite. The ores with which my process is concerned are characterized by such intimate association of magnetite and silica that even when they are ground to exceeding fineness, such as minus 400 mesh for example, a very appreciable amount of silica is still locked or intimately engaged with these fine magnetite particles. The cost of such fine grinding is a very significant factor in the treatment of these ores and militates against their use. Furthermore, even when such ores are finely ground the product of conventional magnetic separation processes is not too desirable because the highest iron content is always associated with the very finest grains and the coarser screen fractions are invariably higher in silica and other gangue materials.

If such ores are to be commercially useful, the middlings which contain most of the silica, although they may represent a relatively small portion of the weight of the ore, must be separated from the finer particles which contain the bulk of the iron. Such a separation is impossible with conventional magnetic separators however because of their non-selective action on mixed particles of magnetite and gangue. These separators attract particles containing 20% magnetite and 80% gangue for example, almost as readily as those containing 80% magnetite and 20% gangue and consequently cannot separate out and divert the middling particles previously mentioned.

It is an object, therefore, of my invention to provide a process for concentrating low grade ores of the character described which makes possible the segregation and diversion of middling particles high in gangue content. It is another object of my invention to provide a process for magnetic concentration of such ores which does not require the extremely fine grinding hitherto considered necessary. Other objects of my invention will appear in the course of the following description.

2

My process may be characterized as a combination of magnetic separation and hydraulic classification. The process of magnetizing finely divided ore before introducing it into a hydraulic classifier is known and it is not to be confused with my process which comprehends hydraulic classification of finely divided particles in a magnetic field. I denominate my process the magnetic reflux concentration of ore and refer to the apparatus employed therein as a magnetic reflux concentrator.

10 In the accompanying drawings, which illustrate a present preferred embodiment of my invention,

Figure 1 is a diagrammatic elevation of a magnetic reflux concentrator and

Figure 2 is a flow sheet illustrating the sequence of procedures comprehended by my process.

My invention will be most readily understood by reference to Figure 1 which illustrates a two-stage magnetic reflux concentrator. Additional stages may be required in a commercial embodiment of my process but their operation will become obvious from the explanation of the two shown. The first stage of this concentrator is designated generally as 1 and the second as 2. The first stage comprises an upright vessel or chamber 4 of non-magnetic material provided with an ore pulp inlet 5, a water inlet 6, an overflow 7 and an underflow pipe 8. The underflow pipe is closed by a valve 9 which may be operated from outside the vessel by means not here shown. A perforated plate 10 is positioned crosswise of the vessel at a point above the water inlet 6, and a magnet 11 surrounds the vessel above the ore pulp inlet 5. This magnet is outside the walls of vessel 4. The second stage of my apparatus is likewise provided with an upright vessel 12 having an ore pulp inlet 13 which communicates with the underflow pipe 8 of the preceding stage, a water inlet 14, an overflow 15, and an underflow pipe 16 provided with a valve 17. A perforated plate 18 corresponds to the similar plate 10 in the first stage 1 and a magnet 19 surrounds the vessel 12 at a region above the pulp inlet 13. The upright chamber 4 with perforated plate 10 and water inlet 6 therebelow comprise the essential features of a hindered settling hydraulic classifier, the conventional operation of which is well known.

In my process iron ore which has been first comminuted and then passed through a conventional wet magnetic separator to remove the free gangue is introduced as an ore pulp through the inlet 5 of the apparatus illustrated. Water under pressure is constantly entering the chamber 4 through the inlet pipe 6, rising through the perforated plate to the top of the chamber and overflowing through the outlet 7. These upwardly flowing currents of water carry the ore pulp upwardly into the region of chamber 4 surrounded by the magnet 11. This magnet, which may be a permanent magnet or an electromagnet energized from a direct current source, not shown, maintains a magnetic field in this portion of the chamber. This magnetic field magnetizes the particles of magnetite contained in the water-borne ore but, of course, does not magnetize the gangue particles. Magnetized ore particles free from gangue are attracted to one another and form rather loosely compacted masses which, because of their weight, tend to sink out of the magnetic field and toward the bottom of the chamber. Particles of ore intimately associated with relatively small amounts of gangue are also attracted in some degree but with a reduced force. This I believe is because the presence of the gangue prevents the magnetite particles closely approaching each other and it is of course known that the force of attraction between magnetized bodies is inversely proportional to the square of the distance between them. Magnetite particles associated with substantial proportions of gangue are not attracted together

with any considerable force and are carried up with the stream of water into the overflow.

The loosely compacted masses of particles attracted together which sink out of the magnetic field are subjected to the upward force of the streams of water rising through the perforated plate which tends to break up these masses and separate those particles bound by lesser attractive forces, that is, the particles containing gangue. These particles when detached from the larger masses are borne upward by the water streams and into the magnetic field where the cycle may be repeated. This reflux is allowed to continue until substantially all particles associated with less than a predetermined amount of gangue sink into the underflow and substantially all those associated with greater amounts are washed out into the overflow. The predetermined separation point depends upon the strength of the magnetic field, which may be adjusted by known ways, such as by adjusting the current supplied to the electromagnet, and the force of the upwardly flowing water, which is easily controlled by a valve. The underflow from the first stage of my process may then be conducted into a second stage which is identical with the first except that the magnetic field and water pressure may be adjusted to different values so that a second fraction of particles associated with gangue is separated and washed out into the overflow. The product of this second stage may, of course, be introduced into additional stages and any desired number of middling fractions separated out. The final product is recovered from the underflow of the last reflux classifier stage. The overflow products of the various stages may be discarded, or recycled as desired. If recycled, the overflow products must pass through a comminution stage to liberate additional iron mineral from the gangue. I prefer to carry out my process in such a way that the overflow from the first stage is higher in gangue than the overflow from the second stage which is higher in gangue than the overflow from the third stage, if any, and so on.

The flow sheet in Figure 2 indicates graphically the sequence of steps of a process utilizing three stages of magnetic reflux concentration as described above.

I have applied the process of my invention successfully to two Michigan iron ores which are not amenable to treatment by conventional concentration processes. These ores, as taken from the mine, exhibit the analyses listed below:

| Ore | Fe, percent | SiO <sub>2</sub> , percent | Fe present as magnetite, percent |
|-----|-------------|----------------------------|----------------------------------|
| A   | 26.97       | 34.18                      | 88.5                             |
| B   | 35.82       | 43.22                      | 86.4                             |

A batch of ore A was ground so that all of it passed through a 100 mesh sieve. It was then processed as indicated by the flow sheet of Figure 2 through a conventional wet magnetic separator and then through a three-stage magnetic reflux concentrator embodying the process of my invention. The composition of the ore entering and leaving the magnetic reflux concentrator and the compositions of the overflow from the three stages are tabulated below:

Table I

| Product                   | Percent Wt. | Percent Fe | Percent SiO <sub>2</sub> | Percent Distribution |                  |
|---------------------------|-------------|------------|--------------------------|----------------------|------------------|
|                           |             |            |                          | Fe                   | SiO <sub>2</sub> |
| Magnetic Separator Output | 100.0       | 53.24      | 14.97                    | 100.0                | 100.0            |
| Conc. Overflow #1         | 5.8         | 11.85      | 45.16                    | 1.3                  | 17.5             |
| Conc. Overflow #2         | 2.8         | 24.78      | 35.94                    | 1.3                  | 6.7              |
| Conc. Overflow #3         | 5.3         | 38.32      | 25.56                    | 3.8                  | 9.1              |
| Underflow                 | 86.1        | 57.87      | 11.60                    | 93.6                 | 66.7             |

It will be observed that the overflow from the first stage of my process contained slightly over 45% SiO<sub>2</sub> which comprised 17.5% of the total amount of SiO<sub>2</sub> of the ore treated. Similarly, the overflow from the second stage analyzed almost 36% SiO<sub>2</sub> which comprised 6.7% of the total SiO<sub>2</sub> introduced. The iron loss in each of these overflows amounted however only to 1.3% of that originally introduced. The final underflow product contained 93.6% of the iron originally present and 66.7% of the silica. This is quite a high recovery of iron and was made possible because the original silica content of the ore was not excessively high.

A batch of ore B was likewise ground so that all of it passed through a 100 mesh sieve and was then concentrated by the process illustrated in the flow sheet of Figure 2. This ore after passing through the wet magnetic separator was considerably higher in silica than ore A. The analyses of this material at various stages of my process are tabulated below:

Table II

| Product                   | Percent Wt. | Percent Fe | Percent SiO <sub>2</sub> | Percent Distribution |                  |
|---------------------------|-------------|------------|--------------------------|----------------------|------------------|
|                           |             |            |                          | Fe                   | SiO <sub>2</sub> |
| Magnetic Separator Output | 100.0       | 54.83      | 22.86                    | 100.0                | 100.0            |
| Conc. Overflow #1         | 6.5         | 20.13      | 62.00                    | 2.4                  | 19.9             |
| Conc. Overflow #2         | 5.1         | 29.61      | 51.38                    | 2.8                  | 13.0             |
| Conc. Overflow #3         | 7.5         | 43.18      | 33.04                    | 5.9                  | 12.2             |
| Underflow                 | 80.9        | 60.29      | 13.74                    | 88.9                 | 54.9             |

It will be observed that my process has recovered 88.9% of the iron in the ore introduced into the magnetic reflux concentrator and has gotten rid of 45.1% of the silica. This is a very satisfactory performance with an ore ground only to minus 100 mesh. If the ore is ground to a smaller size, as is almost always required for previously known processes, a somewhat higher quality concentrate can be produced but this seems to be because the finer grinding enables the conventional wet magnetic separator to remove more of the silica. A batch of ore B ground to minus 200 mesh but otherwise processed as above gave the following results:

Table III

| Product                   | Percent Wt. | Percent Fe | Percent SiO <sub>2</sub> | Percent Distribution |                  |
|---------------------------|-------------|------------|--------------------------|----------------------|------------------|
|                           |             |            |                          | Fe                   | SiO <sub>2</sub> |
| Magnetic Separator Output | 100.0       | 57.98      | 16.23                    | 100.0                | 100.0            |
| Conc. Overflow #1         | 5.9         | 24.86      | 55.78                    | 2.5                  | 20.3             |
| Conc. Overflow #2         | 6.8         | 37.24      | 40.12                    | 4.4                  | 16.8             |
| Conc. Overflow #3         | 4.9         | 51.02      | 24.40                    | 4.3                  | 7.4              |
| Underflow                 | 82.4        | 62.48      | 10.94                    | 88.8                 | 55.5             |

Here again my process brought about a removal of 44.5% of the silica with a recovery of 88.8% of the iron. The results of Tables II and III show that my process does not depend upon costly fine grinding of the ore for its effectiveness.

Although I have described and illustrated a present preferred embodiment of my invention it is not to be considered as limited thereto. My invention is limited only by the appended claims.

65 I claim:

1. The process of treating iron ore composed of heterogeneous fine particles of magnetizable iron mineral associated with gangue comprising carrying the ore particles upwardly in a stream of water into a magnetic field, magnetizing the iron mineral particles, thereby causing them to form by magnetic attraction loosely compacted masses associated with gangue which sink out of the magnetizing field, disintegrating these loosely compacted masses by the stream of water, thereby dissociating gangue particles from iron mineral particles, washing dissociated gangue

particles out in the overflow and collecting iron mineral particles in the underflow.

2. The process of claim 1 in which the strength of the magnetic field and the stream of water are adjusted to disintegrate the loosely compacted masses associated with gangue in excess of a prescribed amount, and iron mineral particles associated with gangue below this prescribed amount are collected in the underflow.

3. The process of claim 1 in which the stream of water is adjusted to disintegrate loosely compacted masses associated with gangue when said masses have sunk out of the magnetic field, but not to disintegrate said masses in the magnetic field.

4. The process of treating iron ore composed of heterogeneous fine particles of magnetizable iron mineral associated with gangue comprising carrying the ore particles upwardly in a stream of water into a magnetic field extending radially about the axis of the stream, magnetizing the iron mineral particles, thereby causing them to form by magnetic attraction loosely compacted free masses associated with gangue which sink out of the magnetizing field, disintegrating these loosely compacted masses by the stream of water, thereby dissociating gangue particles from iron mineral particles, washing dissociated gangue particles out in the overflow and collecting iron mineral particles in the underflow.

5. The process of treating iron ore composed of heterogeneous fine particles of magnetizable iron mineral associated with gangue comprising carrying the ore particles upwardly in a stream of water into a magnetic field, magnetizing the iron mineral particles, thereby causing them to form by magnetic attraction loosely compacted masses associated with gangue which sink out of the magnetizing field, disintegrating these loosely compacted masses by the stream of water, thereby dissociating gangue particles from iron mineral particles, carrying the dissociated iron mineral particles upwardly again into the magnetic field, washing dissociated gangue particles out in the overflow and collecting iron mineral particles in the underflow.

10

15

20

25

30

35

40

6. The process of treating iron ore composed of heterogeneous fine particles of magnetizable iron mineral associated with gangue in a range of intimacies comprising carrying the ore particles upwardly in a stream of water into a magnetic field, magnetizing the iron mineral particles, thereby causing them to form by magnetic attraction loosely compacted masses associated with gangue which sink out of the magnetic field, disintegrating the loosely compacted masses by the stream of water, thereby dissociating from the iron mineral particles gangue particles less intimately associated therewith, carrying the iron mineral particles still associated with gangue upwardly again into the magnetic field, washing dissociated gangue particles out in the overflow and collecting iron mineral particles in the underflow.

#### References Cited in the file of this patent

##### UNITED STATES PATENTS

|           |                  |       |                |
|-----------|------------------|-------|----------------|
| 509,728   | Gillespie        | ----- | Nov. 28, 1893  |
| 827,499   | Bring            | ----- | July 31, 1906  |
| 954,015   | Bent             | ----- | Apr. 5, 1910   |
| 954,016   | Bent             | ----- | Apr. 5, 1910   |
| 1,392,413 | Gow              | ----- | Oct. 4, 1921   |
| 1,491,600 | Fernow           | ----- | Apr. 22, 1924  |
| 2,078,513 | Stearns          | ----- | Apr. 27, 1937  |
| 2,258,194 | Queneau          | ----- | Oct. 7, 1941   |
| 2,276,075 | Wuensch          | ----- | Mar. 10, 1942  |
| 2,309,923 | Robertson        | ----- | Feb. 2, 1943   |
| 2,468,586 | Braund           | ----- | Apr. 26, 1949  |
| 2,558,635 | Vedensky         | ----- | June 26, 1951  |
| 2,563,086 | Verschoor        | ----- | Aug. 7, 1951   |
| 2,612,262 | Symington et al. | ----- | Sept. 30, 1952 |

##### FOREIGN PATENTS

|         |               |       |                |
|---------|---------------|-------|----------------|
| 226,588 | Great Britain | ----- | Dec. 17, 1924  |
| 416,534 | Great Britain | ----- | Sept. 17, 1934 |
| 681,907 | Germany       | ----- | Oct. 4, 1939   |